

# United States Patent [19]

Golborn et al.

[11] 3,895,161

[45] July 15, 1975

[54] FLAME RETARDANT MATERIALS

[75] Inventors: Peter Golborn, Lewiston; James J. Duffy, Buffalo, both of N.Y.

[73] Assignee: Hooker Chemical & Plastics Corporation, Niagara Falls, N.Y.

[22] Filed: Sept. 4, 1973

[21] Appl. No.: 393,868

Related U.S. Application Data

[62] Division of Ser. No. 239,784.

[52] U.S. Cl. .... 428/289; 428/288; 428/378;  
428/921

[51] Int. Cl. .... C09d 5/18

[58] Field of Search .... 117/136, 138.8 B, 143 R,  
117/144, 154, 141; 260/932

[56] References Cited

UNITED STATES PATENTS

|           |        |                |       |           |
|-----------|--------|----------------|-------|-----------|
| 2,666,078 | 1/1954 | Ferguson       | ..... | 117/136 X |
| 2,803,562 | 8/1957 | Erbel et al.   | ..... | 117/136   |
| 2,867,547 | 1/1959 | Fon Toy et al. | ..... | 117/136   |

Primary Examiner—Ralph Husack

Assistant Examiner—Theodore G. Davis

Attorney, Agent, or Firm—Peter F. Casella; Donald C. Studley; William J. Crossetta, Jr.

[57] ABSTRACT

New flame retardant materials are disclosed having applied thereon compounds of the formula:



wherein R is selected from the group consisting of phenyl, lower alkenyl and halogen substituted and unsubstituted lower alkyl of 1-6 carbon atoms, X is selected from the group consisting of chlorine, bromine and lower alkyl of 1-6 carbon atoms, m is an integer from 1-4 and n is an integer from 0-5, provided that the sum of m and n is not greater than 6 and when m is 1, n is greater than 0.

19 Claims, No Drawings

## FLAME RETARDANT MATERIALS

This is a division of application Ser. No. 239,784, filed Mar. 30, 1972, now U.S. Pat. No. 3,803,269 issued Apr. 9, 1974.

## FIELD OF INVENTION

This invention relates to novel compounds of the formula



wherein R is selected from the group consisting of phenyl, lower alkenyl, and halogen substituted and unsubstituted lower alkyl of 1-6 carbon atoms, X is selected from the group consisting of chlorine, bromide and lower alkyl of 1-6 carbon atoms, m is an integer from 1-4 and n is an integer from 0-5, provided that the sum of m and n is not greater than 6 and when m is 1, X is greater than 0. The invention includes methods of applying the above novel compounds to normally flammable textiles, thermoplastic, thermosetting, and elastomeric resin compositions so as to render them flame retardant.

## BACKGROUND OF THE INVENTION

Many flame retarding agents and methods of application have been developed in attempts to obtain flame resistant textile materials and thermoplastic, thermosetting, and elastomeric resin compositions.

Flame retardant textiles have been produced by depositing metal oxides, within or on the textile fibers, by the successive precipitation of ferric oxides and a mixture of tungstic acid and stannic oxide or by successive deposition of antimony trioxide and titanium dioxide. Such processes require plural treatment baths in which strongly acidic solutions are employed thus posing the problem of possible textile degradation. Furthermore, metal oxide coatings on textile materials create difficulties in subsequent dyeing processes which deleteriously affect the hand of the finished product. Another process involves the use of a single processing bath wherein a dispersion of a chlorinated hydrocarbon and finely divided antimony oxide is padded on the textile material. Near the textile combustion temperature antimony oxide will react with hydrogen chloride, generated by degradation of the chlorinated hydrocarbon, to form antimony oxychloride which acts to suppress flame. This combination of a chlorinated hydrocarbon and finely divided antimony oxide are not acceptable finishes for closely woven textiles as they deleteriously affect the hand of the finished product. A further process for imparting flame resistance to cellulosic materials is by the esterification of the cellulose with diammonium hydrogen orthophosphate. Textile products so treated however are subjected to metathesis reaction with cations during washing, and must be regenerated by reacting the wash product with an ammonium chloride solution.

The production of thermoplastic, thermosetting, and elastomeric resin compositions which are flame retardant is of considerable commercial importance. For example, such articles as castings, moldings, foamed or laminated structures and the like are required, or are

at least desired, to be resistant to fire and flame and to possess the ability to endure heat without deterioration. The use of various materials incorporated into thermoplastic, thermosetting and elastomeric resins so as to improve the flame retardancy thereof has been known. Many compounds have been commercially available for such use, among them being chlorostyrene copolymers, chlorinated paraffin wax in admixture with triphenyl styrene, chlorinated paraffins and aliphatic antimonical compounds, as well as antimony oxide-chlorinated hydrocarbon mixtures. A problem associated with these compounds has been however, the fact that generally a large amount, i.e. upwards of 35% of additive, must be incorporated into the resin in order 10 to make it sufficiently flame retardant. Such large amounts of additive may deleteriously affect the physical characteristics of the thermoplastic resin, as well as substantially complicating and increasing the cost of preparation thereof. A further problem is that these 15 prior art additives tend to crystallize or oil out of the resin after a relatively short time of incorporation. The present invention relates to a group of compounds which may be added to thermoplastic resins in relatively small amounts and still produce satisfactory 20 flame retardant compositions which will not crystallize or oil out of the resin after incorporation therein.

## OBJECTS OF THE INVENTION

It is, therefore, a principal object of this invention to 30 provide novel compounds of the formula:



wherein R is selected from the group consisting of phenyl, lower alkenyl and halogen substituted and unsubstituted lower alkyl of 1-6 carbon atoms, X is selected 40 from the group consisting of chlorine, bromine and lower alkyl of 1-6 carbon atoms, m is an integer from 1-4 and n is an integer from 0-5, provided that the sum of m and n is not greater than 6 and when m is 1, X is greater than 0.

It is also an object of this invention to provide flame 45 retarding textile materials comprising normally flammable cellulosic, proteinaceous or analogous man-made materials. Another object is to provide a method for treating normally flammable cellulosic, proteinaceous or analogous man-made materials to render them flame retardant. Another object is to provide 50 flame retarding thermoplastic, thermosetting or elastomeric resin compositions comprising normally flammable resin materials. A further object is to provide a process for treating normally flammable thermoplastic, thermosetting or elastomeric resin compositions to render them flame retardant. A particular object is to devise a composition comprising normally flammable cellulosic, proteinaceous or analogous man-made materials and an effective flame retardant amount of the compound represented by the formula



wherein R, X, m and n are as above described.

A further particular object is to devise a composition comprising normally flammable thermoplastic, thermo-setting or elastomeric polymers and an effective flame retarding amount of the before described novel compound.

These and other objects of the present invention will be obvious from the following description.

#### DESCRIPTION OF THE INVENTION

In accordance with this invention there are provided novel compounds, for imparting flame retardancy to textiles and resin materials, of the formula



wherein R is selected from the group consisting of phenyl, lower alkenyl and halogen substituted and unsubstituted lower alkyl of 1-6 carbon atoms, X is selected from the group consisting of chlorine, bromine and lower alkyl of 1-6 carbon atoms, m is an integer from 1-4 and n is an integer from 0-5, provided that the sum of m and n is not greater than 6 and when m is 1, X is greater than 0.

10 More specifically, the preferred compounds of the present invention include these compounds wherein R is lower alkyl, alkenyl chlorinated alkyl or phenyl, and X is chlorine, bromine or methyl.

15 Illustrative examples of compounds of the present invention include, for instance, compounds of the general formula such as





This synthesis of the compositions of the present invention is accomplished by reacting on N-hydroxymethyl aromatic amides of the formula



with a trialkyl phosphate of the formula



wherein R, m, n and X are as previously described in a suitable solvent, excess of the phosphate or neat. Typically, the reaction occurs at elevated temperatures and is continued for about 1 to about 12 hours. Temperatures are generally about 50°C to about 160°C. Preferably reaction is continued from about 3 to about 6 hours at a temperature of about 80°C to about 120°C. The solvent or other volatiles is thereafter stripped, or otherwise removed from the product. Suitable solvents include benzene, toluene, xylene, glymes, dimethylformamide, aliphatic or aromatic hydrocarbons. Typical N-hydroxymethyl aromatic amides operable as reactants herein include



One or more of the novel compounds of this invention may be applied to textile materials by conventional finishing techniques such as by thermal induced pad curing so as to incorporate into the textile a flame retardant amount thereof. The compounds of this invention have advantages over the flame retardant agents of the prior art in that they may be used on a variety of textile materials of different chemical composition, and

they may be applied by a variety of methods. They may be applied to materials in either the fiber or fabric form to give flame retarding materials with minimum detectable physical changes in the quality or hand of the textile material.

Cellulosic textile materials may be made flame retardant by way of a variety of methods. Products of this invention may be applied to cellulosic materials in several ways to give a durable flame retardant treatment.

- 10 For example, the products of this invention may be reacted with formaldehyde to give N-hydroxymethyl derivatives which can react with cellulosic materials in a known manner. Alternatively aqueous mixtures of the products with formaldehyde, urea, trimethylol melamine or other known cellulose crosslinking agents may be applied to a cellulose substrated with the aid of an acidic catalyst by a pad dry process.

More preferably the N-hydroxymethyl derivative of the products of this invention prepared by the condensation of the products with formaldehyde, are mixed in an aqueous medium with trimethylol melamine and a Lewis acid catalyst such as  $\text{NH}_4\text{Cl}$  or  $\text{Zn}(\text{NO}_3)_2 \cdot 6\text{H}_2\text{O}$ .

- 25 The cellulosic material is immersed in a aqueous solution of the methyl derivative, trimethylol melamine, and  $\text{Zn}(\text{NO}_3)_2 \cdot 6\text{H}_2\text{O}$  and squeezed on a two roll padder to 70-90% wet weight pick-up. The material is dried at 220°-270°F for 1-3 minutes and cured at 300°-370°F for 1-6 minutes in a circulating air oven. The samples are then washed in hot water and dried. The finished samples have a flame retardant add on of about 5 to about 40% and preferably about 10 to about 25% by weight.

30 The flame retardant agents of this invention may be applied to various textiles such as cellulosic materials, proteinaceous materials and blends of cellulosic or proteinaceous materials and analogous manmade fibers. By cellulosic materials, applicant intends to embrace cotton, rayon, paper, regenerated cellulose and cellulose derivatives which retain a cellulose backbone of at least one hydroxy substituent per repeating glucose unit. By proteinaceous material applicant intends to embrace those textile materials comprising the functional groups of proteins such as the various animal wools, hairs and furs.

- 35 The flame retardant compounds or additives of the invention may be incorporated into thermoplastic, thermosetting or elastomeric resin compositions by any known method. That is to say, the flame retardant additive may be added to the resin by milling the resin and the additive on, for example, a two-roll mill, or in a Banbury mixer etc., or it may be added by molding or extruding the additive and resin simultaneously, or by merely blending it with the resin in powder form and thereafter forming the desired article. Additionally, the flame-retardant may be added during the resin manufacture, i.e., during the polymerization procedure by which the resin is made, provided the catalysts etc. and other ingredients of the polymerization system are inert thereto. Generally, the compounds of this invention may be incorporated into the thermoplastic resin in flame-retarding amounts, i.e. generally amounts ranging from about 5% by weight, to about 50% by weight, preferably from about 20% by weight, to about 40% by weight, based on the weight of the polymer, have been found sufficient.

60 Resins embraced within the scope of this invention include the homopolymers and copolymers of unsaturated aliphatic, alicyclic, and aromatic hydrocarbons.

Suitable monomers are ethylene, propylene, butene, pentene, hexene, heptene, octene, 2-methylpropene-1, 3-methylbutene-1, 4-methylpentene-1, 4-methylhexene-1, 5-methylhexene-1, bicyclo-(2.2.1)-2-heptene, butadiene, pentadiene, hexadiene, isoprene, 2,3-dimethylbutadiene-1,3, 2-methylpentadiene-1,3, 4-vinylcyclohexene, vinylcyclohexene, cyclopentadiene, styrene and methylstyrene, and the like.

Other polymers in addition to the above-described olefin polymers that are useful in the invention include polyindene, indenecoumarone resins; polymers of acrylate esters and polymers of methacrylate esters, acrylate and methacrylate resins such as ethyl acrylate, n-butyl methacrylate, isobutyl methacrylate, ethyl methacrylate and methyl methacrylate; alkyd resins and paint vehicles, such as bodied linseed oil; cellulose derivatives such as cellulose acetate, cellulose acetate butyrate, cellulose nitrate, ethyl cellulose, hydroxyethyl cellulose, methyl cellulose and sodium carboxymethyl cellulose; epoxy resins; furan resins (furfuryl alcohol or furfuralketone); hydrocarbon resins from petroleum; isobutylene resins (polyisobutylene); isocyanate resins (polyurethanes); melamine resins such as melamine-formaldehyde and melamine-urea-formaldehyde; oleoresins; phenolic resins such as phenol-formaldehyde, phenolic-elastomer, phenolic-epoxy, phenolic-polyamide, and phenolic-vinyl acetals; polyamide polymers, such as polyamides, polyamide-epoxy and particularly long chain synthetic polymeric amides containing recurring carbonamide groups as an integral part of the main polymer chain; polyester resins such as unsaturated polyesters of dibasic acids and dihydroxy compounds, and polyester elastomer and resorcinol resins such as resorcinol-formaldehyde, resorcinol-furfural, resorcinol-phenol-formaldehyde, resorcinol-polyamide and resorcinol-urea; rubbers such as natural rubber, synthetic polyisoprene, reclaimed rubber, chlorinated rubber, polybutadiene, cyclized rubber, butadiene-acrylonitrile rubber, butadiene-styrene rubber, and butyl rubber; neoprene rubber (polychloroprene); polysulfides (Thiokol); terpene resins; urea resins; vinyl resins such as polymers of vinyl acetal, vinyl acetate or vinyl alcohol-acetate copolymer, vinyl alcohol, vinyl chloride, vinyl butyral, vinyl chloride-acetate copolymer, vinyl pyrrolidone and vinylidene chloride copolymers; polyformaldehyde; polyphenylene oxide; polymers of diallyl phthalates and phthalates; polycarbonates of phosgene or thiophosgene and dihydroxy compounds such as bisphenols phosgene, thermoplastic polymers of bisphenols and epichlorohydrin (trade named Phenoxy polymers); graft copolymers and polymers of unsaturated hydrocarbons and unsaturated monomer, such as graft copolymers of polybutadiene, styrene and acrylonitrile, commonly called ABS resins; ABS polyvinyl chloride polymers, recently introduced under the trade name of Cycovin; and acrylic polyvinyl chloride polymers, known by the trade name Kydex 100.

The polymers of the invention can be in various physical forms, such as shaped articles, for example, moldings, sheets, rods, and the like; fibers, coatings, films and fabrics, and the like.

The compounds of this invention have been found to have particular utility in ABS resins and in elastomeric materials such as acrylic rubber; acrylonitrile-butadiene styrene terpolymers; butadiene-acrylonitrile copolymers; butyl rubber; chlorinated rubbers, e.g., polyvinyl chloride resins, chloroprene rubber, chloro-

sulfonated polyethylene; ethylene polymers, e.g., ethylene-propylene copolymers, ethylene-propylene terpolymers; fluorinated rubbers, butadiene rubbers, e.g., styrene-butadiene rubber, isobutylene polymers, polybutadiene polymers, polyisobutylene rubbers, polyisoprene rubbers; polysulfide rubbers; silicon rubbers; urethane rubbers; high styrene resins latices, high styrene resins, vinyl resins; sponge rubber; and the like.

It should be noted that it is also within the scope of 10 the present invention to incorporate such ingredients as plasticizers, dyes, pigments, stabilizers, antioxidants, antistatic agents and the like to the novel composition.

ASTM Test D2863-70, used in accordance with the following examples, generally provides for the comparison of relative flammability of self-supporting plastics 15 by measuring the minimum concentration of oxygen in a slowly rising mixture of oxygen and nitrogen that will support combustion. The procedure encompasses supporting cylindrical test specimens 70-150 mm  $\times$  8.0 mm vertically in a glass tube fitted with controlled upward oxygen-nitrogen gas flow. The top of the specimen is ignited and oxygen flow is adjusted until it reaches that minimum rate at which the specimen is extinguished before burning 3 minutes or 50 mm which ever happens first. The oxygen index(*n*) is then calculated as follows:

$$n, \% = (100 \times O_2) / (O_2 + N_2)$$

wherein  $O_2$  is the volumetric flow of oxygen, at the minimal rate and  $N_2$  is the corresponding volumetric flow rate of nitrogen.

A modification of ASTM Test D635-68 used in accordance with the following examples, generally provides for the comparison of burning rates, self-extinguishment and non-burning characteristics of plastics in the form of sheets, bars, plates or panels. The procedure encompasses preparing plastic samples of 150-200 mm  $\times$  8 mm with and without the subject 35 flame additive. Each sample is marked at points 1 inch and 4 inches from its end and held, marked end in the flame, at a 45° angle in a controlled burner flame (1 inch flame length) for two 30 second attempts. The movement of the flame up the length of the sample through the two points is measured for rate of burning, 40 non-burning or self-extinguishing characteristics. A sample is rated SE(self-extinguishing) if the flame burns through the first point but extinguishes before reaching the second point. A sample is rated NB(non-burning) if, upon ignition it does not burn to the first 45 point.

AATCC test method 34-1969, The Vertical Char Test, used in accordance with the following examples, generally provides for the comparison of relative flammability of 2 1/4 inch  $\times$  10 inch fabric test specimens 55 when exposed to a controlled burner flame, under controlled conditions, for periods of 12.0 and 3.0 seconds. Charred specimens are thereafter subjected to control tearing tests, using tabulated weights, to determine the average tear length as representing the char length of the fabric. In addition, samples which are wholly consumed by the flame are rated (B) and samples which do not burn are rated (NB). For comparison purposes, it should be noted that untreated samples of the fabrics used in the examples of this case would be consumed 60 for this test.

In all the examples of the application, the following general procedure was used except when otherwise specifically noted. Padding was done on a standard two

roll laboratory padder at a gauge pressure of about 60 pounds per square inch in all cases. Drying and curing during processing were done with a standard laboratory textile circulating air oven. Washing and drying was done in a standard, home, top loading, automatic washer and dryer.

The following examples are set forth for purposes of illustration only and are not to be construed as limitations of the present invention except as set forth in the appended claims. All parts and percentages are by weight unless otherwise specified.

## EXAMPLE I

## Preparation of



A 500 ml. flask was charged with 124g. (1.0 mole) of trimethyl phosphite and was heated to about 100°C. 57.5g. (0.25 mole) of 3-bromo-N-hydroxymethyl benzamide was then added to the reaction flask over a period of 5 minutes. The reaction mixture was then refluxed at about 95° for about 3 hours then stripped at 100°C under a vacuum of 0.5 mm mercury to give 81g of a colorless, viscous oil which by elemental analysis was confirmed to be the desired product.

## EXAMPLE II

## Preparation of



Following the procedure described in Example I 69g. (0.3 mole) of 3-bromo-N-hydroxymethyl benzamide was refluxed with 80g. (0.35 mole) of tri-n-butyl phosphite for about 5 hours at about 125°C. n-Butanol and excess tri-n-butyl phosphite were removed by stripping the reaction mixture at 115°C under a vacuum of 0.5 mm mercury. After stripping 121g. of a pale yellow viscous liquid was obtained which was confirmed, by elemental analysis to be the desired product.

## EXAMPLE III

## Preparation of



A 500 ml. flask, fitted with a reflux condenser, mechanical stirrer and thermometer, was charged with 124g. (1.0 mole) of trimethyl phosphite and was heated to about 100°C. 61.8g. (0.3 mole) of 2,4-dichloro-N-hydroxymethyl benzamide was added to the trimethyl phosphite, over a period of about 5 minutes. The homogeneous reaction mixture was then refluxed at about 93°C for 3 hours and thereafter stripped, under a reduced pressure of about 0.5 mm Hg. at about 10°C, to give 93g. of a tacky solid. Recrystallization of the solid

5

from benzene of cyclohexane (1:1) gave 82.8g. of dimethyl 2,4-dichlorobenzamidomethyl phosphonate.

## EXAMPLE IV

## Preparation of



A 250 ml. flask was charged with 62g. (0.5 mole) of trimethyl phosphite and was heated to about 100°C. 29g. (0.1 mole) of bis-N,N-hydroxymethyl tetrachloroterephthalamide was added to the flask and the reaction mixture was refluxed for about 6 hours and then cooled to room temperature. Unreacted solids were filtered off and the filtrate was stripped, at 70°C under 2 mm. mercury of reduced pressure, to give 12.0g. of a tacky solid product which was found, by infrared and nuclear magnetic resonance spectroscopy to be substantially pure desired product.

15

## Preparation of



A 250 ml. flask was charged with 21.9g. (0.1 mole) of 2,4-dichloro-N-hydroxymethyl benzamide and 27g. (0.1 mole) of tris-2-chloroethyl phosphite. This reaction mixture was heated at about 130°C for about 4 hours then stripped, at 100°C under a vacuum of 1.3 mm mercury, to give 41 grams of a white solid. The product was proven, by elemental and infrared and nuclear magnetic resonance spectroscopy, to be substantially pure desired product.

20

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

## 10

from benzene of cyclohexane (1:1) gave 82.8g. of dimethyl 2,4-dichlorobenzamidomethyl phosphonate.

## EXAMPLE IV

## Preparation of



A 250 ml. flask was charged with 62g. (0.5 mole) of trimethyl phosphite and was heated to about 100°C. 29g. (0.1 mole) of bis-N,N-hydroxymethyl tetrachloroterephthalamide was added to the flask and the reaction mixture was refluxed for about 6 hours and then cooled to room temperature. Unreacted solids were filtered off and the filtrate was stripped, at 70°C under 2 mm. mercury of reduced pressure, to give 12.0g. of a tacky solid product which was found, by infrared and nuclear magnetic resonance spectroscopy to be substantially pure desired product.

## EXAMPLE V

## Preparation of



A 250 ml. flask was charged with 21.9g. (0.1 mole) of 2,4-dichloro-N-hydroxymethyl benzamide and 27g. (0.1 mole) of tris-2-chloroethyl phosphite. This reaction mixture was heated at about 130°C for about 4 hours then stripped, at 100°C under a vacuum of 1.3 mm mercury, to give 41 grams of a white solid. The product was proven, by elemental and infrared and nuclear magnetic resonance spectroscopy, to be substantially pure desired product.

20

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

A 500 ml. flask, equipped with mechanical stirrer, thermometer and reflux condenser, was charged with 66g (0.4 mole) of N-hydroxymethyl p-toluamide and 124 g (1.0 mole of trimethyl phosphite. This reaction mixture was refluxed for about 4 hours then stripped, at 70°C under 0.2 mm mercury vacuum, to give 95g of a low melting solid. Elemental analysis with infrared and nuclear magnetic resonance spectroscopy confirmed the structure of the product.

## EXAMPLE VIII

## Preparation of



Triphenyl phosphite (62g, 0.2 mole), was mixed with N-hydroxymethyl-p-toluamide in a 250 ml. round bottomed three necked flask fitted with mechanical stirrer, thermometer, and reflux condenser. The mixture was warmed to and maintained at about 130°C for about 5 hours. After cooling the mixture was stripped, at 120°C and 2 mm Hg, to remove phenol and other volatile material. The stripping product was identified by elemental analysis as N-(diphenylphosphonomethyl)-p-toluamide and was obtained in 85.3% yield.

## EXAMPLE IX

## Preparation of



A mixture of 44.8g (0.2 mole) of N,N'-bis-hydroxyphenyl terephthalamide and 124 g (1.0 mole) of trimethyl phosphite was refluxed for about 6 hours. After the completion of the reaction the mixture was stripped, at 120°C and 1 mm Hg, to remove excess phosphite and other volatiles. The product was confirmed by infrared and nuclear magnetic resonance spectroscopy.

## EXAMPLE X

## Preparation of

- 12
- 5 A mixture of 60.3g of triallyl phosphite and 22.4g of N,N'-bis-hydroxymethyl terephthalamide was heated at about 130°C for about 6 hours. The reaction mixture was stripped, at 100°C and 1 mm Hg, to remove all volatile materials. A yellow liquid, which weighed 62.0g, 10 was isolated and confirmed as the desired product by spectroscopic and elemental analyses.

## EXAMPLE XI

- 15 Forty parts of N-dimethylphosphonomethyl-2,4-dichlorobenzamide was mixed with 60 parts of polypropylene and dry blended for about five minutes. This mixture was then heated to a melt and mixed well in the molten state for about 15 minutes. The mixture was 20 then allowed to cool to room temperature and the plastic composition was cut into small pieces. These pieces were placed slowly into a glass tube (9 mm) immersed in a hot metal bath, the temperature of the bath being maintained above the melt temperature of the plastic composition. Pieces of the composition were added until the melt had a depth of approximately 200 mm. A metal rod was then placed in the tube with a weight attached and the tube cooled to solidify the composition. The composition was then removed from the tube 25 and tested by ASTM tests D2863-70 and D635-68. The results of the testing are contained in Table 1.

## EXAMPLES XII-XXIX

- 35 Various additive compounds were mixed and treated 35 with various resins according to the method of Example XI. Table 1 tabulates the results of testing by ASTM tests D2863-70 and D635-68 for Examples XII-XXIX.

## EXAMPLE XXX

- 40 N-Dimethyl phosphonomethyl-p-toluamide (25g) was mixed with 40% formalin solution (37.5g) and stirred overnight at pH 10. The pH was adjusted to 7.0 with hydrochloric acid and 3.1g of ammonium chloride and 14.0g of a 50% solution of a methylolated melamine added. 5.0 oz. sq. yd. cotton sheeting was immersed in the solution and the excess squeezed from the cloth by passing through a two roll laboratory padder at 60 lb. gauge pressure, to a wet pick-up of about 90%. The sheeting was then dried at about 250°F for 45 about 2 minutes and cured at about 340°F for about 5 minutes in a circulating air oven. The sheeting was then washed by hand for about 5 minutes in a detergent (Tide) water mixture and tumble dried. A resin pick-up of 23.7% was calculated.
- 55

TABLE I

| Example | Polymer                    | Additive | Percent Additive (By Weight) | Flammability Tests |       |
|---------|----------------------------|----------|------------------------------|--------------------|-------|
|         |                            |          |                              | O1                 | D-635 |
| XI      | Polypropylene              |          | 40                           | 19.8               | SE    |
| XII     | Nylon                      |          | 30                           | 26.6               | NB    |
| XIII    | Polyethylene Terephthalate |          | 30                           | 28                 | NB    |

TABLE I-Continued

| Example | Polymer                    | Additive | Percent Additive (By Weight) | Flammability Tests |       |
|---------|----------------------------|----------|------------------------------|--------------------|-------|
|         |                            |          |                              | OI                 | D-635 |
| XIV     | ABS                        |          | 30                           | 24                 | NB    |
| XV      | Nylon                      | ditto    | 30                           | 25                 | NB    |
| XVI     | Polyethylene Terephthalate | ditto    | 30                           | 36                 | NB    |
| XVII    | ABS                        |          | 40                           | 22.3               | SE    |
| XVIII   | Nylon                      | ditto    | 40                           | 26                 | NB    |
| XIX     | Epoxy                      | ditto    | 30                           | 29                 | NB    |
| XX      | Polystyrene                |          | 30                           | 23.3               | SE    |

TABLE I (continued)

| Example | Polymer                    | Additive | Percent Additive (By Weight) | Flammability Tests |       |
|---------|----------------------------|----------|------------------------------|--------------------|-------|
|         |                            |          |                              | OI                 | D-635 |
| XXI     | Polyethylene Terephthalate |          | 40                           | 29.4               | NB    |
| XXII    | Epoxy                      |          | 30                           | 24.7               | SE    |
| XXIII   | Epoxy                      |          | 30                           | 28                 | SE    |
| XXIV    | Polyethylene Terephthalate | ditto    | 30                           | 27.5               | SE    |
| XXV     | ABS                        | ditto    | 40                           |                    | SE    |
| XXVI    | Polystyrene                |          | 40                           |                    | SE    |
| XXVII   | ABS                        | ditto    | 30                           | 24.3               |       |
| XXVIII  | Polystyrene                |          | 40                           | 23.8               |       |
| XXIX    | SBR                        | ditto    | 30                           | 24.1               | SE    |

The then treated sheeting was thereafter subjected to ASTM test D2863-70 and AATCC test 34-1969 with initial results as indicated in Table II. The cotton sheeting was thereafter subjected to four additional hand washes, as above described, and tested under AATC test 34-1969.

#### EXAMPLES XXXI-XXXIII

Using the method of Example 30, 5 oz. per sq. yard cotton sheeting was treated with various compounds and subjected to ASTM test D2863-70 and AATCC test 34-1969. The results therefore are indicated in Table II.

#### EXAMPLE XXXIV

Rayon staple fiber was immersed in the solution described in Example XXX and squeezed on a two roll laboratory padder at about 60 lb. gauge pressure to a wet pick-up of about 100%. The fiber was then dried for about 3 minutes at about 250°F and cured for about 10 minutes at about 350°F in a circulating air oven. The fiber was then washed by hand for about 5 minutes in a hot detergent (Tide) water mixture and dried in the circulating air oven resulting in an add-on of about 13.8%. The fiber was then tested for flammability by holding one end of a treated sample in a benson flame

for about 2 sec. and then removing and observing the sample. Treated samples self-extinguish immediately while untreated samples are completely consumed.

The fiber was then further tested for durability by subjecting it to a 5 complete wash cycles in a standard, home type automatic washer using Tide detergent. Thereafter the fiber was tested for flammability as previously described. The results of testing is tabulated in Table II.

## EXAMPLES XXXV-XXXVI

Using the method of Example XXXIV, rayon staple fiber was treated with various compounds and subjected to ASTM test D2863-70 and AATCC test 34-1969. The results are shown in Table II.

## EXAMPLE XXXVII

N-Diallyl phosphonomethyl-p-toluamide (19g) was mixed with 40% formalin solution (28.5g) and stirred overnight at pH 10. The pH was brought to 7.0 with hydrochloric acid and ammonium chloride (2.4g) and a 50% solution of a methylolated malamine (10.9g) added.

6.0 oz. sq. yd. wool was immersed in the above solution, squeezed on a 2 roll laboratory padder to a wet pick-up of about 100% dried for about 2 minutes at about 250°F and cured for about 5 minutes at about 350°F in a circulating air oven. The wool was then washed for one wash cycle using Tide, in a standard, home type, automatic washer and tumble dried. The resin add-on was calculated as 25.3%.

The thus treated wool was thereafter subjected to ASTM test D2863-70 and AATCC test 34-1969. The wool was then subjected to four additional one cycle washings in a standard home type automatic washer, as above described, and thereafter tested by AATCC test 34-1969. Test results are tabulated in Table II.

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035<br

5. The textile material of claim 1 wherein said compound is:



6. The textile material of claim 1 wherein said compound is:



7. The textile material of claim 1 wherein said compound is:



8. The textile material of claim 1 wherein said compound is:



9. The textile material of claim 1 wherein said compound is:



10. The textile material of claim 1 wherein said compound is:



11. The textile material of claim 1 wherein said compound is:



12. The textile material of claim 1 wherein said compound is:



35 13. The textile material of claim 1 wherein said compound is:



45 14. The fire retardant textile material of claim 1  
wherein about 5 to about 40% by weight of said com-  
pound has been added on.

15. The fire retardant textile material of claim 1 wherein about 10 to about 25% by weight of said compound has been added on.

50 16. The fire retardant textile material of claim 1 wherein said compound is applied by padding.

17. The fire retardant textile material of claim 1 wherein said compound is applied to thermal induced pad curing.

55 18. The fire retardant textile material of claim 1  
wherein said compound is applied to the textile mate-  
rial while in the fiber form.

19. The fire retardant textile material of claim 1 wherein said compound is applied to the textile material in fabric form.

\* \* \* \* \*

60 \* \* \* \* \*

\* \* \* \*